

[54] SILVER HALIDE SUPERSENSITIZED PHOTOGRAPHIC EMULSION

[75] Inventors: Keisuke Shiba; Akira Sato, both of Kanagawa, Japan

[73] Assignee: Fuji Photo Film Co., Ltd., Kanagawa, Japan

[\*] Notice: The portion of the term of this patent subsequent to Feb. 27, 1990, has been disclaimed.

[22] Filed: Jan. 10, 1973

[21] Appl. No.: 322,581

## Related U.S. Application Data

[63] Continuation-in-part of Ser. No. 49,981, June 25, 1970, Pat. No. 3,718,475.

## [30] Foreign Application Priority Data

June 25, 1969 Japan ..... 44-50118

[52] U.S. Cl. ..... 96/124

[51] Int. Cl. ..... G03c 1/14

[58] Field of Search ..... 96/124

## [56] References Cited

## UNITED STATES PATENTS

|           |        |              |       |        |
|-----------|--------|--------------|-------|--------|
| 3,666,480 | 5/1972 | Shiba et al. | ..... | 96/124 |
| 3,713,835 | 1/1973 | Sato et al.  | ..... | 96/124 |
| 3,718,475 | 2/1973 | Shiba et al. | ..... | 96/124 |

Primary Examiner—J. Travis Brown

Attorney, Agent, or Firm—Sughrue, Rothwell, Mion, Zinn &amp; Macpeak

## [57] ABSTRACT

A silver halide photographic emulsion is super-

sensitized in the green wave length region by adding thereto at least one sensitizing dye of the following formula I and at least one sensitizing dye of the following formula II; and, optionally a compound of the following formula III:



The substituents are described in detail hereinbelow.

15 Claims, 12 Drawing Figures

PATENTED NOV 19 1974

3,849,147

SHEET 1 OF 2

**FIG. 1**



**FIG. 2**



**FIG. 3**



**FIG. 4**



**FIG. 5**



**FIG. 6**



FIG. 7



FIG. 9



FIG. 8



FIG. 10

FIG. 11



FIG. 12



## SILVER HALIDE SUPERSENSITIZED PHOTOGRAPHIC EMULSION

## CROSS-REFERENCE TO RELATED APPLICATIONS

The present application is a continuation-in-part of Ser. No. 49,981 filed June 25, 1970, now U.S. Pat. No. 3,718,475.

## BACKGROUND OF THE INVENTION

## 1. Field of the Invention

This invention relates to a super-sensitized silver halide photographic emulsion and more particularly it relates to a super-sensitized silver halide photographic emulsion for increasing particularly the spectral sensitivity in the green region. Furthermore, the invention relates to a super-sensitized silver halide photographic emulsion containing couplers for making color photographic light-sensitive materials.

## 2. Description of the Prior Art

It is well known that a spectral sensitizing method is one of the techniques employed in the manufacture of silver halide photographic emulsions, and that the sensitizing method is an indispensable technique for the production of color photographic light-sensitive materials. The spectral sensitivity obtained by the method is influenced not only by the chemical structure of the sensitizing dye to be used and the properties of the silver halide emulsion to be used, such as the composition of the halogen and the crystal system of the silver halide contained in the emulsion, the manner of chemical ripening, the silver ion concentration and the hydrogen ion concentration of the emulsion, but also by the various kinds of additives added to the silver halide emulsion.

In many cases, the spectral sensitivity is reduced. However, when a certain kind of sensitizing dye is used together with a dye or a colorless aromatic compound having a specific chemical structure according to the chemical structure and the properties of the sensitizing dye, a higher spectral sensitivity is obtained than when using each of the sensitizing dyes alone. This is known as a super-sensitizing action.

In particular, silver halide emulsions used for producing color photographic light-sensitive materials contain a large amount of couplers, and when a coupler is incorporated in a silver halide photographic emulsion containing a sensitizing dye, the spectral sensitivity becomes lower than the spectral sensitivity obtained by using the sensitizing dye alone. In addition, the presence of the coupler reduces the super-sensitizing action.

Also, the spectral sensitivity distribution in the green region, in which man's visual sensitivity is high, is one of the most important factors for the color reproduction of color photographic light-sensitive materials and for the quality of the image obtained.

Therefore, various studies have been made concerning the sensitization of silver halide emulsions in the green region. For example, a method of using a combination of a benzimidazolocarbocyanine dye and a pseudocyanine dye is described in the specification of U.S. Pat. No. 2,701,198. However, when the method described in the aforementioned U.S. patent is applied to a silver halide emulsion containing a coupler, only a lower sensitivity is obtained due to the presence of the coupler in the emulsion.

Also, a method of using a combination of a benzimidazolo carbocyanine dye and a benzoxazolocarbocyanine dye is described in the specification of Japanese Pat. Publication No. 4936/68. However, this method has the disadvantages that the sensitivity in the shorter wave length side of the green region, e.g., in a wave length region of 500-530 m $\mu$  is large, and also the contamination effect by the dyes after development is large.

10 Therefore, a primary object of the present invention is to provide a silver halide photographic emulsion having both a high spectral sensitivity in a wave length region of 500-530 m $\mu$  and less of a contamination by the dyes after development.

15 Another object of the present invention is to provide a silver halide photographic emulsion used for producing a color photographic light-sensitive material having a high green sensitivity in the presence of a coupler.

## SUMMARY OF THE INVENTION

The above objects of the present invention can be attained by super-sensitizing a silver halide photographic emulsion with at least one sensitizing dye represented by the following formula I:



35 wherein R<sub>1</sub> and R<sub>2</sub> which may be the same or different) each represents an alkyl group, an aryl group or a substituted alkyl group; R<sub>3</sub> and R<sub>4</sub> (which may be the same or different) each represents an alkyl group, an aryl group, a substituted alkyl group, a sulfoalkyl group or (preferably) a substituted alkyl group having a sulfo group of the formula: -alkyl-(R<sub>8</sub>)-SO<sub>3</sub><sup>-</sup> or



45 wherein  $R_8$  is an atomic group and  $n$  is an integer of at least 1, at least one of said  $R_3$  and  $R_4$  being a sulfoalkyl group or said substituted alkyl group having a sulfo group and the end carbon atom of the alkyl moiety of the sulfoalkyl group or said substituted alkyl group having a sulfo group forming a covalent bond with the nitrogen atom of the heterocyclic nucleus;  $Z_1$  and  $Z_2$  (which may be the same or different) each represents a non-metallic atomic group necessary to complete a substituted or unsubstituted heterocyclic nucleus of the benzimidazole series;  $X_1^-$  represents an acid anion group of the type usually employed in cyanine dyes; and  $p$  is an integer of 1 or 2,  $p$  being 1 when the cyanine dye of formula I forms an intermolecular salt; and at least one of the sensitizing dyes represented by the following formula II:



wherein  $Z_3$  represents a non-metallic atomic group necessary to complete a substituted or unsubstituted heterocyclic nucleus of the 2-quinoline series;  $Z_4$  represents a non-metallic atomic group necessary to complete a benzoxazole nucleus, a naphthoxazole nucleus, a benzthiazole nucleus, a benzselenazole nucleus, a naphthothiazole nucleus, or a naphthoselenazole nucleus, each being unsubstituted or substituted by an alkyl group, a trifluoromethyl group, a halogen atom, an alkoxy group or sulfoalkoxy group;  $R_5$  and  $R_6$  (which may be the same or different) each represents an alkyl group, a substituted alkyl group having a sulfo group as defined above (in  $R_3$  and  $R_4$ ), other substituted alkyl groups or a sulfoalkyl group; at least one of said  $R_5$  and  $R_6$  being a sulfoalkyl group or said substituted alkyl group having a sulfo group except where the heterocyclic nucleus containing  $Z_4$  has been substituted by a sulfoalkoxy group;  $X_2^-$  represents an acid anion group of the type usually employed in cyanine dyes; and  $q$  is an integer of 1 or 2,  $q$  being 1 when the cyanine dye of formula II forms an intermolecular salt.

Furthermore, it has been discovered according to the present invention that a particularly better result is obtained by incorporating a compound represented by the following formula II in the above-mentioned silver halide photographic emulsion.



wherein  $R_7$  represents an alkyl group or a substituted alkyl group;  $Z_5$  represents a non-metallic atomic group necessary to complete a substituted or unsubstituted heterocyclic nucleus of the benzimidazole series; and  $Z_6$  represents a phenyl group or a substituted phenyl group, such as a phenyl group substituted by alkyl groups, alkoxy groups, and the like.

#### BRIEF DESCRIPTION OF THE DRAWINGS

The Figures are spectograms showing the relative sensitivity (i.e., speed) of various photographic films employing super-sensitizing dye combinations according to the present invention as well as prior art combinations and individual dyes alone.

#### DETAILED DESCRIPTION OF THE PREFERRED EMBODIMENTS

As stated above, at least one of  $R_3$  and  $R_4$  is a sulfoalkyl group or, preferably, said substituted alkyl group having a sulfo group of the formula indicated. The atomic group represented by  $R_{68}$  may be, for example, an alkoxy group, an alkylamino group, an alkoxyamino

group or a thioalkoxy group and, preferably,  $n$  is a positive integer of up to 2.

The end carbon atom of the alkyl group (i.e., the " $-C$ " in " $-CH_2CH_2CH_2SO_3^-$ ") forms a covalent bond with the nitrogen atom of the heterocyclic nucleus.

Typical examples of the preferred  $R_3$  and  $R_4$  groups are: sulfoalkoxyalkyl groups, sulfoalkoxyalkoxyalkyl groups and sulfohydroxyalkyl groups (i.e.,  $-alkyl-alkoxy-SO_3^-$ ,  $-alkoxy-alkoxy-alkoxy-SO_3^-$  and



In the above-mentioned formulae I and II, the alkyl groups of  $R_1$  to  $R_7$  include: methyl, ethyl, n-propyl, isopropyl, n-butyl and iso-butyl groups; and as the substituted alkyl groups of  $R_1$  to  $R_6$  there may be illustrated: an allyl group, an aralkyl group, a  $\beta$ -acetoxy-ethyl group, a  $\gamma$ -acetoxypropyl group, a  $\gamma$ -carboxypropyl group, a  $\beta$ -carboxyethyl group, a  $\gamma$ -sulfatopropyl group, a  $\delta$ -sulfatobutyl group, a  $\delta$ -N-acetylsulfamyl butyl group and a  $\beta$ -hydroxyethyl group.

Examples of the sulfoalkyl group of  $R_3$  -  $R_6$  are a  $\beta$ -sulfopropyl group, a  $\beta$ -sulfonylbutyl group or a  $\delta$ -sulfobutyl group;

Examples of said substituted alkyl group having a sulfo group of  $R_3$  and  $R_4$  are a 2-(3-sulfopropoxy)ethyl group, a 2-[2-(3-sulfopropoxy) ethoxy]ethyl group, and a 2-hydroxy-1-sulfopropyl group.

As the benzimidazole series nucleus completed by  $Z_1$ ,  $Z_2$  or  $Z_5$ , there may be illustrated: benzimidazole and benzimidazole containing, as a component of the skeletal-structure thereof, a benzene ring substituted by at least one of the following: a halogen atom, an N-unsubstituted or alkyl substituted sulfamyl or carbamyl group, an N-disubstituted sulfamyl group such as a morpholino sulfonyl group, an alkyl sulfonyl group, a trifluoromethyl group, an unsubstituted or substituted alkyl group, the substituent being an aralkyl group (e.g., benzyl) or a carboxyalkyl group (e.g., carboxymethyl), a cyano group, a phenyl group, a carboalkoxyl group, a hydroxyl group, and an alkoxy group.

Also, the 2-quinoline series nucleus completed by  $Z_3$  in the above-mentioned formula II may be, for example, 2-quinoline and 2-quinoline containing, as a component of the skeletal-structure thereof, a benzene ring substituted by at least one of the following: an alkyl group and a halogen atom.

The substituted alkyl group  $R_7$  in the above-mentioned formula III is, for example, a sulfoalkyl group neutralized by a cation, such as alkali metal ions, organic ammonium ions, a pyridinium ion, a benzylthiuronium ion, and the like, i.e., a cation of the type usually employed in cyanine dyes, a cyanoalkyl group and an allyl group,

As  $X_1$  and  $X_2$  in the formulae I and II, there may be illustrated e.g., a halogen, perchlorate, thiocyanate, p-toluene sulfonate, benzene sulfonate, methyl sulfate and ethyl sulfate ions.

The sensitizing dye represented by formula II has at least one sulfo group in the heterocyclic nucleous containing  $Z_4$  or at  $R_5$  or  $R_6$ . The spectral sensitizing obtained by using the sensitizing dye represented by formula II (i.e., a monomethine cyanine dye) is ordinarily reduced by the introduction of a sulfo group therein. Therefore, it is quite surprising that when the sensitizing dye represented by formula I is used together therewith, the spectral sensitization is increased.

The sensitizing dye represented by the formula II may be substituted therein by an alkyl group, a phenyl group, a halogen atom, an alkoxy group, or an alkoxy group substituted by at least a sulfo group; in other words, the substituent is so selected that the maximum sensitivity obtained by using at least one sensitizing dye of formula II and at least one compound of formula I

in combination does not shift to a longer wave length side than that of the sensitizing dye of formula II.

The compound represented by formula III shows a super-sensitizing action to the sensitizing dye represented by formula I and to the sensitizing dye represented by formula II, and by using the compound represented by formula III together with the combination of the other two sensitizing dyes, the green sensitivity is further increased and at the same time the sensitivity in the wave length region of 500-530 m $\mu$ , which is present at a shorter wave length side of the green region, is further increased.

The compounds which may be used in the present invention will be further illustrated by reference to the following illustrative formulae, which are merely illustrative, and not limiting, in nature.







The above-mentioned sensitizing dyes or the other compounds which may be used in this invention may be synthesized by known methods.

For instance, they can be synthesized by the methods described in the specifications of U.S. Pat. Nos. 2,503,776 and 2,778,823; Belgian Pat. Nos. 590,607; 704,296; 668,014; 669,133; 669,934; 673,554; and 697,006; British Pat. Nos. 742,112; 955,964; 975,504; and 980,234; Japanese Pat. Publication Nos. 14112/65; 23467/65; and 13823/68; and Japanese Pat. Application Nos. 55439/67 and 76071/67.

Also, other sensitizing dyes and the compounds used in this invention, which were not described above, may also be easily synthesized by referring to the specifications of the above patents.

The compounds used in this invention are incorporated in a silver halide emulsion as solutions in water or a water-soluble organic solvent such as methanol, etha-

nol, and pyridine. The sensitizing dyes represented by formula I and formula II, respectively, may be added to a silver halide emulsion as a mixture of the solutions thereof or as separate solutions. The amounts of these dyes are greatly influenced by the nature of the silver halide emulsion to be used. usually, the total amount of the above-mentioned sensitizing dyes (I and II) and compound III are preferably from  $1 \times 10^{-6}$  mol to  $1 \times 10^{-3}$  mol, per mol of silver halide. The weight ratio of the amount of the sensitizing dye represented by formula II to the amount of the sensitizing dye represented by formula I is preferably from 10:1 to 1:2, but this ratio is varied by the amount, 1/10 to 5 times by mole based on dye I, of the compound represented by formula III to be added.

As the silver halide emulsion which may be used in this invention, there may be illustrated: a silver iodobromide emulsion, a silver bromide emulsion, a silver

chlorobromide emulsion, etc. The silver halide emulsion used in this invention is mainly a gelatino silver halide emulsion but the emulsion may contain, besides gelatin, polyvinyl alcohol, an alginic acid polymer, polyvinyl imidazole, polyvinyl pyrrolidone, or copolymers thereof, or may be an emulsion thereof.

The silver halide emulsion of this invention is applied to a suitable support according to the desired use, such as a paper, a glass plate, a cellulose triacetate film, a polyethylene terephthalate film, other plastic films than above, a baryta-coated paper, a resin-coated paper, or a synthetic paper.

The present invention will be illustrated further by the following examples which are merely illustrative and not limited in nature.

### EXAMPLE 1

50 g of 1-phenyl-3-[3-(2,4-di-tertiaryamylphenoxyacetamido)-benzamido]5-pyrazolone was dissolved in 100 ml of dibutyl phthalate by heating and the resultant solution was added to 1 liter of a 10 percent aqueous gelatin solution. Then, 50 ml of a 5 percent aqueous solution of sodium alkylbenzene sulfonate was added thereto and they were dispersed by emulsification by means of a high speed rotary mixer (the product is called the dispersion of the magenta coupler).

1 kg. of a silver iodobromide emulsion (containing 0.25 mol of silver and 4.0 mol percent of iodine) prepared by a conventional method was placed in a beaker and melted at 40°C. After adding to the emulsion the sensitizing dye in the amounts shown in Table 1, the emulsion was stirred for 15 minutes. Further, 400 g. of the dispersion of the magenta coupler as prepared above was added to the emulsion with stirring and after adding further suitable amounts of a hardening agent and an ampholite surface active agent as a wetting agent to the mixture with stirring, the resultant mixture was applied to a cellulose triacetate film in a thickness of 7 microns to obtain a sample of a green-sensitive light-sensitive material.

The sample was cut into strips and subjected to an optical wedge exposure through Yellow Filter No. K-12 made by Fuji Photo Film Co. by using a sensitometer of 5,400°K in color temperature of the light source. The strip thus exposed was developed for 12 minutes at 20°C in a color developer having the following composition:

|                              |         |
|------------------------------|---------|
| N,N-diethyl-p-aminobenzoate  | 2.9 g   |
| Sodium sulfite               | 2.0 g   |
| Sodium carbonate monohydrate | 50.0 g  |
| Hydroxylamine hydrochloride  | 1.5 g   |
| Potassium bromide            | 1.0 g   |
| Water to make                | 1000 ml |
| (pH, 10.8 ± 0.1)             |         |

Thereafter, the strip was further processed in a first fixing solution, a bleaching solution and a second fixing solution and washed with water to obtain a magenta image. After drying the sample strips thus processed, the green filter density was measured by using an S-type Densitometer made by Fuji Photo Film Co., from which characteristic curves were obtained. From these results, the densities at the point of fog plus 0.20 were calculated and the results are shown in Table 1.

The compositions of the bleaching solution and the fixing solution used in the above processing were as follows:

### Composition of the Bleaching Solution

|                   |         |
|-------------------|---------|
| Ferricyanide      | 100 g   |
| Potassium bromide | 20 g    |
| Water to make     | 1000 ml |
| (pH, 6.9 ± 0.3)   |         |

### Composition of the Fixing Solution

|                   |         |
|-------------------|---------|
| Hypo              | 200 g   |
| Sodium sulfite    | 20 g    |
| Acetic acid (28%) | 45 ml   |
| Boric acid        | 7.5 g   |
| Potassium alum    | 20 g    |
| Water to make     | 1000 ml |
| (pH, 4.5 ± 0.2)   |         |

TABLE I

| Dye  | Amount (ml)<br>(mol concen-<br>tration) | Dye   | Amount (ml)<br>(mol concen-<br>tration) | (A) | (B)  |
|------|-----------------------------------------|-------|-----------------------------------------|-----|------|
| (IA) | 40( $5 \times 10^{-4}$ )                |       | —                                       | 115 | 0.17 |
|      | 80                                      |       | —                                       | 120 | 0.23 |
|      | 40                                      | (IIC) | 20( $1 \times 10^{-3}$ )                | 142 | 0.18 |
|      | do.                                     |       | 40                                      | 165 | 0.20 |
|      | do.                                     |       | 120                                     | 158 | 0.23 |
|      | —                                       |       | 40                                      | 43  | 0.11 |
|      | —                                       |       | 120                                     | 50  | 0.12 |
|      | —                                       |       | —                                       | 100 | 0.13 |
|      | —                                       |       | —                                       | 100 | 0.15 |
|      | —                                       | (IIA) | 40( $1 \times 10^{-3}$ )                | 200 | 0.25 |
| (IB) | 49( $5 \times 10^{-4}$ )                |       | 80                                      | 186 | 0.25 |
|      | 80                                      |       | —                                       | 35  | 0.13 |
|      | 40                                      |       | 80                                      | 35  | 0.13 |
|      | do.                                     |       | 80                                      | 220 | 0.21 |
|      | —                                       |       | 40                                      | 282 | 0.25 |
|      | —                                       |       | 40                                      | 43  | 0.13 |
|      | —                                       |       | 80                                      | 46  | 0.13 |
|      | —                                       |       | 80                                      | 190 | 0.23 |
|      | —                                       |       | 80                                      | 220 | 0.25 |
|      | —                                       |       | 40                                      | 33  | 0.11 |
| (IC) | 40( $5 \times 10^{-4}$ )                |       | 80                                      | 35  | 0.12 |
|      | 80                                      |       | —                                       | 105 | 0.13 |
|      | 40                                      | (IIE) | 40( $5 \times 10^{-4}$ )                | 105 | 0.15 |
|      | do.                                     |       | 80                                      | 200 | 0.19 |
|      | do.                                     |       | 80                                      | 220 | 0.20 |
|      | —                                       |       | 160                                     | 220 | 0.22 |
|      | —                                       |       | 40                                      | 45  | 0.18 |
|      | —                                       |       | 80                                      | 50  | 0.17 |
|      | —                                       |       | 160                                     | 58  | 0.15 |
|      | —                                       |       | 40                                      | 252 | 0.24 |
| (IE) | 40( $5 \times 10^{-4}$ )                |       | 40                                      | 282 | 0.27 |
|      | 80                                      |       | 80                                      | 218 | 0.26 |
|      | 40                                      |       | 20                                      | 50  | 0.22 |
|      | do.                                     |       | 40                                      | 60  | 0.22 |
|      | —                                       |       | 80                                      | 60  | 0.22 |
|      | —                                       |       | —                                       | 110 | 0.18 |
|      | —                                       |       | —                                       | 115 | 0.24 |
|      | —                                       |       | 80                                      | 200 | 0.20 |
|      | —                                       |       | 80                                      | 234 | 0.21 |
|      | —                                       |       | 40                                      | 25  | 0.17 |
| (ID) | 40( $1 \times 10^{-3}$ )                |       | 80                                      | 25  | 0.18 |
|      | 118                                     |       | 0.18                                    | —   | —    |
|      | 80                                      |       | —                                       | 118 | 0.14 |
|      | 40                                      | (IIH) | 40( $5 \times 10^{-4}$ )                | 250 | 0.17 |
|      | do.                                     |       | 80                                      | 316 | 0.20 |
|      | —                                       |       | 40                                      | 33  | 0.15 |
|      | —                                       |       | 80                                      | 40  | 0.15 |
|      | —                                       |       | —                                       | 100 | 0.15 |
|      | —                                       |       | —                                       | 115 | 0.22 |
|      | —                                       |       | 40                                      | 200 | 0.20 |
| (IG) | 40( $5 \times 10^{-4}$ )                |       | do.                                     | 220 | 0.25 |
|      | 80                                      |       |                                         | 79  | 0.25 |
|      | 40                                      | (IIB) | 40( $1 \times 10^{-3}$ )                | 85  | 0.27 |
|      | do.                                     |       | 80                                      | 118 | 0.27 |
|      | —                                       |       | 40                                      | 150 | 0.30 |

(A): Relative yellow filter sensitivity (S<sub>y</sub>)

(B): Fog.

### EXAMPLE 2

As in Example 1, 1 kg of a silver iodobromide emulsion (containing 0.30 mol of silver and 6.0 mol percent of iodine) was melted in a beaker at 40°C and the amounts of the sensitizing dyes I and II and the compound of formula III shown in Table 2 were added to the emulsion with stirring. 7 ml of the silver halide

emulsion thus obtained was applied to a glass plate of cabinet size followed by drying to obtain a sample.

The sample was cut into strips and the strips were subjected to an optical wedge exposure by yellow light as in Example 1 and then developed in a developer having the following composition for 10 minutes at 20°C.

| Composition of the Developer |         |
|------------------------------|---------|
| Water                        | 500 ml  |
| Metol                        | 0.3 g   |
| Sodium pyrosulfite           | 38 g    |
| Hydroquinone                 | 6 g     |
| Sodium carbonate monohydrate | 22.5 g  |
| Citric acid                  | 0.7 g   |
| Potassium bromide            | 0.9 g   |
| Water to make                | 1000 ml |

The strips were then fixed and the optical densities thereof were measured, the results of which are shown in Table 2.

TABLE 2

| Dye | Amount (ml)<br>(mol concen-<br>tration) | Dye | Amount (ml)<br>(mol concen-<br>tration) | Compd | Amt (ml)<br>(mol concen-<br>tration) | A    | B    |
|-----|-----------------------------------------|-----|-----------------------------------------|-------|--------------------------------------|------|------|
| IB  | 40( $5 \times 10^{-4}$ )                | —   | —                                       | —     | 100                                  | 0.15 |      |
| do. | 80 do.                                  | —   | —                                       | —     | 97                                   | 0.16 |      |
| do. | 40 do.                                  | IIB | 40( $1 \times 10^{-3}$ )                | —     | 142                                  | 0.15 |      |
| do. | do.                                     | do. | 80 do.                                  | —     | 178                                  | 0.16 |      |
| do. | do.                                     | do. | 60 do.                                  | IIIA  | 20( $1 \times 10^{-3}$ )             | 166  | 0.15 |
| do. | do.                                     | do. | do.                                     | do.   | 40 do.                               | 200  | 0.15 |
| do. | do.                                     | do. | do.                                     | do.   | 80 do.                               | 200  | 0.16 |
| do. | do.                                     | do. | do.                                     | IIIB  | 40( $1 \times 10^{-3}$ )             | 178  | 0.16 |
| do. | do.                                     | do. | do.                                     | do.   | 80 do.                               | 190  | 0.16 |
| do. | do.                                     | do. | do.                                     | IIIC  | 40( $1 \times 10^{-3}$ )             | 190  | 0.16 |
| do. | do.                                     | do. | do.                                     | do.   | 80 do.                               | 200  | 0.17 |

(A): Relative yellow filter sensitivity (Sy)

(B): Fog

The strips were then fixed and the optical densities thereof measured. In addition, the fog values of the developed strips were also measured.

The structure of the dyes employed are shown hereinbelow, and the amounts of the various dyes in each samples as well as the measured sensitivity and fog values are shown in Table 3 below.

Table 3

| Dyes<br>ml (mole concentration) |                           | Dyes<br>ml (mole concentration) |                           | Yellow Filtered Relative<br>Sensitivity | Fog Spectrogram     |
|---------------------------------|---------------------------|---------------------------------|---------------------------|-----------------------------------------|---------------------|
| (IB)                            | 80 ( $5 \times 10^{-4}$ ) | —                               | —                         | 100                                     | 0.11                |
| do.                             | 160                       | —                               | —                         | 96                                      | 0.12                |
| (A)                             | 40 ( $5 \times 10^{-4}$ ) | —                               | —                         | 79                                      | 0.11                |
| do.                             | 80                        | —                               | —                         | 84                                      | 0.12                |
| do.                             | 160                       | —                               | —                         | 69                                      | 0.14                |
|                                 |                           | (IIJ)                           | 80 ( $2 \times 10^{-3}$ ) | 33                                      | 0.10                |
|                                 |                           |                                 | 160                       | 33                                      | 0.10                |
|                                 |                           | (B)                             | 80 ( $2 \times 10^{-3}$ ) | 47                                      | 0.11                |
|                                 |                           |                                 | 160                       | 47                                      | 0.11                |
| (IB)                            | 80 ( $5 \times 10^{-4}$ ) | (IIJ)                           | 40 ( $2 \times 10^{-3}$ ) | 211                                     | 0.09                |
| do.                             | 80                        | —                               | 80                        | 225                                     | 0.12 FIG. 1 curve 1 |
| (A)                             | 80 ( $5 \times 10^{-4}$ ) | (B)                             | 40 ( $2 \times 10^{-3}$ ) | 157                                     | 0.12                |
| do.                             | 80                        | —                               | 80                        | 157                                     | 0.16 FIG. 2 curve 2 |

## EXAMPLE 3

A silver bromoiodide emulsion was prepared by a conventional method such that one kilogram of the resulting silver halide emulsion had a silver content of 0.6 mole and an iodide content of 6.0 mole percent. Various samples were made by the following procedure.

One kilogram of the above-produced silver bromoiodide emulsion was weighed into a beaker and melted in a water-bath at 40°C. To the melted emulsion, certain amounts of sensitizing dyes were added with stirring, the amounts and type of dyes being shown in the table below. Seven milliliters of the resulting emulsion were weighed and coated onto a cabinet size glass plate to obtain samples.

Each sample was cut into strips and subjected to an optical wedge exposure through a yellow filter, No.

## 14

K-12, made by Fuji Photo Film Co., Ltd. employing a sensitometer having a light source of 5.400°K in color temperature. The exposed strips were then developed for 10 minutes at 200°C in a developer having the following composition:

5

## Composition of the Developer

|    |                              |      |    |
|----|------------------------------|------|----|
| 10 | Water                        | 500  | ml |
|    | Metol                        | 0.3  | g  |
|    | Sodium pyrosulfite           | 38   | g  |
|    | Hydroquinone                 | 6    | g  |
|    | Sodium carbonate monohydrate | 22.5 | g  |
|    | Citric acid                  | 0.7  | g  |
|    | Potassium bromide            | 0.9  | g  |
|    | Water to make                | 1000 | ml |

15

The strips were then fixed and the optical densities thereof measured. In addition, the fog values of the developed strips were also measured.

The structure of the dyes employed are shown hereinbelow, and the amounts of the various dyes in each samples as well as the measured sensitivity and fog values are shown in Table 3 below.



**EXAMPLE 4**

As in Example 1, 1 kg of a silver iodobromide emulsion containing 0.52 mol of silver and 7 mol percent of iodine wherein an average grain diameter of the silver halide is  $0.78 \mu$  was weighed into a beaker and melted in a bath at  $40^\circ\text{C}$  and the amounts of the sensitizing dyes I and II shown in Table 4 were added to the emulsion. To the resulting emulsion there were added 10 ml of 1 percent by weight aqueous solution of sodium 1-hydroxy-3,4-dichlorotriazine and 10 ml of a 2 percent by weight aqueous solution of sodium nonyl benzene sulfonate and then the emulsion thus obtained was applied to a cellulose triacetate film base in a thickness of 5 microns (in a dried state) to obtain a sample.

The sample was cut into strips and subjected to an optical wedge exposure through a yellow filter according to Example 1. The strips were then developed and fixed, and the optical densities thereof were measured according to Example 2, the results of which are shown in Table 4 below.

In addition, spectrograms were obtained according to conventional procedures by means of a spectrophotometer having a light source of 2,666°K and a reflection type-defraction lattice.

Table 4

| Dye  | Dye Amount(ml)<br>(Mol Concentration) |                      | Dye    | Dye Amount(ml)<br>(Mol Concentration) |                      | (A) | (B)  | Spectrogram |          |
|------|---------------------------------------|----------------------|--------|---------------------------------------|----------------------|-----|------|-------------|----------|
| (IB) | 40                                    | $(5 \times 10^{-4})$ |        |                                       | —                    | 100 | 0.05 |             |          |
|      | 80                                    |                      |        |                                       | —                    | 80  | 0.06 | FIG. 3      | curve 1  |
|      |                                       | —                    | (IIK)  | 80                                    | $(1 \times 10^{-3})$ | 32  | 0.08 |             |          |
| (IB) | 80                                    | $(5 \times 10^{-4})$ | (IIK)  | 160                                   |                      | 40  | 0.06 | do.         | 2        |
| do.  |                                       | —                    |        | 80                                    |                      | 138 | 0.09 |             |          |
|      |                                       | —                    |        | 160                                   |                      | 160 | 0.10 | do.         | 3        |
| (IB) | 80                                    | $(5 \times 10^{-4})$ | (III)  | 80                                    | $(1 \times 10^{-3})$ | 89  | 0.10 | FIG. 4      | curve 4  |
|      | 80                                    | —                    |        | 160                                   |                      | 96  | 0.14 |             |          |
| (IB) | 80                                    | $(5 \times 10^{-4})$ | (III)  | 80                                    |                      | 152 | 0.09 | do.         | 5        |
|      | 80                                    | —                    |        | 160                                   |                      | 152 | 0.12 |             |          |
| (IB) | 80                                    | $(5 \times 10^{-4})$ | (IIIM) | 80                                    | $(1 \times 10^{-3})$ | 63  | 0.07 | FIG. 5      | curve 6  |
|      | 80                                    | —                    |        | 160                                   |                      | 63  | 0.10 |             |          |
| (IB) | 80                                    | $(5 \times 10^{-4})$ | (IIIM) | 80                                    |                      | 178 | 0.11 | do.         | 7        |
|      | 80                                    | —                    |        | 160                                   |                      | 167 | 0.11 |             |          |
|      |                                       | (D)                  |        | 80                                    | $(1 \times 10^{-3})$ | 44  | 0.06 | FIG. 6      | curve 8  |
|      |                                       |                      |        | 160                                   |                      | 44  | 0.11 |             |          |
| (IB) | 80                                    |                      | (D)    | 80                                    |                      | 117 | 0.08 | do.         | 9        |
| (A)  | 80                                    |                      | (D)    | 80                                    |                      | 112 | 0.36 | do.         | 10       |
| (ID) | 40                                    | $(5 \times 10^{-4})$ |        |                                       |                      | 100 | 0.07 | FIG. 11     | curve 11 |
|      | 80                                    |                      |        |                                       |                      | 112 | 0.08 |             |          |
|      |                                       |                      | (IIIN) | 80                                    | $(1 \times 10^{-3})$ | 32  | 0.06 |             |          |
|      |                                       |                      |        | 160                                   |                      | 32  | 0.06 |             |          |
| (ID) | 80                                    | $(5 \times 10^{-4})$ | (IIIO) | 80                                    | $(1 \times 10^{-3})$ | 160 | 0.10 | FIG. 11     | curve 12 |
| do.  |                                       | —                    |        | 160                                   |                      | 200 | 0.12 |             |          |
| (IB) | 80                                    | $(5 \times 10^{-4})$ | (IIIN) | 80                                    | $(1 \times 10^{-3})$ | 160 | 0.10 | FIG. 12     | curve 13 |
| do.  |                                       | —                    |        | 160                                   |                      | 178 | 0.10 |             |          |
|      |                                       | (IIIO)               |        | 80                                    | $(1 \times 10^{-3})$ | 40  | 0.08 |             |          |
|      |                                       |                      |        | 160                                   |                      | 62  | 0.08 |             |          |

Dyes A and D shown in Table 4 have the following structures:



### EXAMPLE 5

A silver bromoiodide emulsion was prepared by a conventional method such that one kilogram of the resulting silver halide emulsion had a silver content of 0.6 mole and an iodide content of 6.0 mole percent. Various samples were made by the following procedure.

10 One kilogram of the above-produced silver bromoiodide emulsion was weighed into a beaker and melted in a water-bath at 40°C. To the melted emulsion, certain amounts of sensitizing dyes were added with stirring, the amounts and type of dyes being shown in the table below. Seven milli liters of the resulting emulsion were 15 weighed and coated onto a cabinet size glass plate to obtain samples.

Each sample was cut into strips and subjected to an optical wedge exposure through a yellow filter, No. 20 K-12, made by Fuji Photo Film Co., Ltd. employing a sensitometer having a light source of 5,400°K in color temperature. The exposed strips were then developed for 10 minutes at 200°C in a developer having the following composition:

### Composition of the Developer

|                              |         |
|------------------------------|---------|
| Water                        | 500 ml  |
| Metol                        | 0.3 g   |
| Sodium pyrosulfite           | 38 g    |
| Hydroquinone                 | 6 g     |
| Sodium carbonate monohydrate | 22.5 g  |
| Citric acid                  | 0.7 g   |
| Potassium bromide            | 0.9 g   |
| Water to make                | 1000 ml |

The strips were then fixed and the optical densities thereof measured. In addition, the fog values of the developed strips were also measured.

The structure of the dyes employed are shown here-  
 65 inbelow, and the amounts of the various dyes in each sample as well as the measured sensitivity and fog values are shown in Table 5 below.

TABLE 5

|      | Dyes<br>ml (mole concentration) | Dyes<br>ml (mole concentration) | Yellow<br>filtered<br>Relative<br>Sensitivity | Fog  | Spectrogram     |
|------|---------------------------------|---------------------------------|-----------------------------------------------|------|-----------------|
| (IB) | 80 ( $5 \times 10^{-4}$ )       |                                 | 100                                           | 0.12 |                 |
|      | 160                             |                                 | 95                                            | 0.13 |                 |
| (A)  | 40 ( $5 \times 10^{-4}$ )       |                                 | 79                                            | 0.11 |                 |
|      | 80                              |                                 | 84                                            | 0.12 |                 |
|      | 160                             |                                 | 70                                            | 0.13 |                 |
|      |                                 | (IIJ) 80 ( $2 \times 10^{-3}$ ) | 32                                            | 0.10 |                 |
|      |                                 | 160                             | 32                                            | 0.10 |                 |
|      |                                 | (B) 80 ( $2 \times 10^{-3}$ )   | 47                                            | 0.10 |                 |
|      |                                 | 160                             | 47                                            | 0.10 |                 |
| (IB) | 80 ( $5 \times 10^{-4}$ )       | (IIJ) 40 ( $2 \times 10^{-3}$ ) | 210                                           | 0.10 |                 |
|      | 80 ( $5 \times 10^{-4}$ )       | 80                              | 225                                           | 0.12 | FIG. 7, curve 1 |
| (IB) | 80 ( $5 \times 10^{-4}$ )       | (B) 40 ( $2 \times 10^{-3}$ )   | 166                                           | 0.10 |                 |
|      | 80 ( $5 \times 10^{-4}$ )       | 80                              | 166                                           | 0.11 | FIG. 7, curve 2 |
| (A)  | 80 ( $5 \times 10^{-4}$ )       | (IIJ) 40 ( $2 \times 10^{-3}$ ) | 132                                           | 0.09 | FIG. 8, curve 3 |
|      | 80 ( $5 \times 10^{-4}$ )       | 80                              | 157                                           | 0.11 |                 |
| (A)  | 80 ( $5 \times 10^{-4}$ )       | (B) 40 ( $2 \times 10^{-3}$ )   | 158                                           | 0.12 | FIG. 8, curve 4 |
|      | 80 ( $5 \times 10^{-4}$ )       | 80                              | 157                                           | 1.15 |                 |

## EXAMPLE 6

A silver bromoiodide emulsion was prepared as set forth in Example 5 above, and various amounts of the same dyes in the same amounts as shown in Table 6 were added to different emulsions. To each spectrally sensitized silver bromoiodide emulsion was added, with stirring, 600 grams of the magenta coupler dispersion described in Example 1. To each of the resulting emul-

image. The compositions of the bleaching solution and fixing solution are shown in Example 1. After drying each sample strip as processed above, the green filter density was measured employing an S-type densitometer made by Fuji Photo Film Co., Ltd., from which the characteristic curves of each sample were obtained. From these results, the densities at the point of fog plus 0.20 were calculated and the results are shown in Table 6 below:

TABLE 6

|      | Dyes<br>ml (mole concentration) | Dyes<br>ml (mole concentration) | Yellow<br>Filtered<br>Relative<br>Sensitivity | Fog  | Spectrogram        |
|------|---------------------------------|---------------------------------|-----------------------------------------------|------|--------------------|
| (IB) | 80 ( $5 \times 10^{-4}$ )       |                                 | 89                                            | 0.13 |                    |
|      | 160                             |                                 | 96                                            | 0.11 |                    |
| (A)  | 40 ( $5 \times 10^{-4}$ )       |                                 | 70                                            | 0.10 |                    |
|      | 80                              |                                 | 89                                            | 0.11 |                    |
|      | 160                             |                                 | 89                                            | 0.14 |                    |
|      |                                 | (IIJ) 80 ( $2 \times 10^{-3}$ ) | 25                                            | 0.11 |                    |
|      |                                 | 160                             | 27                                            | 0.11 |                    |
|      |                                 | (B) 80 ( $2 \times 10^{-3}$ )   | *                                             | 0.10 |                    |
|      |                                 | 160                             | *                                             | 0.11 |                    |
| (IB) | 80 ( $5 \times 10^{-4}$ )       | (IIJ) 40 ( $2 \times 10^{-3}$ ) | 170                                           | 0.11 |                    |
|      | 80 ( $5 \times 10^{-4}$ )       |                                 | 220                                           | 0.14 | FIG. 9<br>Curve 5  |
| (IB) | 80 ( $5 \times 10^{-4}$ )       | (B) 40 ( $2 \times 10^{-3}$ )   | 95                                            | 0.11 | FIG. 9<br>Curve 6  |
|      | 80 ( $5 \times 10^{-4}$ )       | 80                              | 95                                            | 0.11 |                    |
| (A)  | 80 ( $5 \times 10^{-4}$ )       | (IIJ) 40 ( $2 \times 10^{-3}$ ) | 135                                           | 0.11 | FIG. 10<br>Curve 7 |
|      | 80 ( $5 \times 10^{-4}$ )       | 80                              | 142                                           | 0.21 |                    |
| (A)  | 80 ( $5 \times 10^{-4}$ )       | (B) 40 ( $2 \times 10^{-3}$ )   | 74                                            | 0.11 | FIG. 10<br>Curve 8 |
|      | 80 ( $5 \times 10^{-4}$ )       | 80                              | 77                                            | 0.11 |                    |

\*difficult to determine a sensitivity

sions were added a hardening agent and an anionic surface-activating agent, as is conventional, and the resulting emulsions were coated onto a cellulose triacetate film base to obtain green-sensitive photographic materials. The resulting samples were cut into strips and subjected to an optical wedge exposure through a yellow filter, No. K-12, made by Fuji Photo Film Co., Ltd., employing a sensitometer whose light source had a color temperature of 5,400°K. Each exposed strip was developed for 12 minutes at 20°C in a color developer having the following composition:

|                                   |         |
|-----------------------------------|---------|
| N,N-diethyl-p-aminobenzoate       | 2.0 g   |
| Sodium sulfite                    | 2.0 g   |
| Sodium carbonate monohydrate      | 50 g    |
| Hydroxylamine hydrochloride       | 1.5 g   |
| Potassium bromide                 | 1.0 g   |
| Water to make<br>(pH, 10.8 ± 0.1) | 1000 ml |

Thereafter, each strip was further processed in a first fixing solution, a bleaching solution and a second fixing solution and washed with water to maintain a magenta

What is claimed is:

1. A super-sensitized silver halide photographic emulsion wherein the light-sensitivity in the wavelength region of 500-530 m $\mu$  is increased containing at least one first sensitizing dye represented by the following formula I:



wherein  $\text{R}_1$  and  $\text{R}_2$ , which may be the same or different, each represents an alkyl group, an aryl group or a substituted alkyl group with the substituent being vinyl, aryl, acetoxy, carboxy, sulfato, N-acetylsulfamyl or hydroxy;  $\text{R}_3$  and  $\text{R}_4$ , which may be the same or different, each represents an alkyl group, a substituted alkyl

group with the substituents being the same as in the substituted alkyl group of  $R_1$  and  $R_2$ , an aryl group, a sulfoalkyl group or a substituted alkyl group having a sulfo group of the formula



wherein  $R_8$  represents an atomic group and  $n$  is an integer of at least 1; at least one of said  $R_3$  and  $R_4$  being sulfoalkyl or said substituted alkyl group having a sulfo group, the end carbon atom of said sulfoalkyl group or said substituted alkyl group having a sulfo group forming a covalent bond with the nitrogen atom of the heterocyclic nucleus;  $Z_1$  and  $Z_2$ , which may be the same or different, each represents a non-metallic atomic group necessary to complete a heterocyclic nucleus of the benzimidazole series, said nucleus being unsubstituted or substituted with halogen, an N-unsubstituted or alkyl-substituted sulfamyl or carbamyl group, an N-disubstituted sulfamyl group, an alkyl sulfonyl group, a trifluoromethyl group, an alkyl group, a substituted alkyl group wherein the substituent is an aryl group or a carboxyl group, a cyano group, a phenyl group, a carboalkoxyl group, a hydroxyl group or an alkoxy group;  $X_1^-$  represents an acid anion group and  $p$  is an integer of 1 or 2, being 1 when the dye of formula I forms an intermolecular salt; and at least 1 second sensitizing dye represented by the following formula II:



wherein  $Z_3$  represents a non-metallic atomic group necessary to complete a substituted or unsubstituted heterocyclic nucleus of the 2-quinoline series wherein the substituent is alkyl or halogen;  $Z_4$  represents a non-metallic atomic group necessary to complete a benzoxazole nucleus, a naphthoxazole nucleus, a benzthiazole nucleus, a benzelenazole nucleus, a naphthothiazole nucleus or a naphthoelenazole nucleus, each of said nuclei being unsubstituted or substituted by an alkyl group or a trifluoromethyl group, a phenyl group, a halogen atom, an alkoxy group or an alkoxy group having a sulfo group;  $R_5$  and  $R_6$ , which may be the same or different each represents an alkyl group, a substituted alkyl group with the substituents being the same as in the substituted alkyl group of  $R_1$  and  $R_2$ , a sulfoalkyl group or said substituted alkyl group having a sulfo group; at least one of said  $R_5$  and  $R_6$  being a sulfoalkyl group or said substituted alkyl group having a sulfo group except where the heterocyclic nucleus completed by  $Z_4$  has been substituted by a sulfoalkoxyl group;  $X_2^-$  represents an acid anion; and  $q$  is an integer of 1 or 2,  $q$  being 1 when the dye of formula II forms an intermolecular salt.

2. A super-sensitized silver halide emulsion according to claim 1 wherein said silver halide emulsion further contains a compound represented by the following formula III:

Formula III



wherein  $R_7$  represents an alkyl group or a substituted alkyl group wherein the substituent is a sulfoalkyl group neutralized by a cation, a cyano group or a vinyl group;  $Z_5$  represents an atomic group necessary to complete a heterocyclic nucleus of the benzimidazole series, said nucleus being unsubstituted or substituted with halogen, an N-unsubstituted or alkyl-substituted sulfamyl or carbamyl group, an N-disubstituted sulfamyl group, an alkyl sulfonyl group, a trifluoromethyl group, an alkyl group, a substituted alkyl group wherein the substituent is an aryl group or a carboxyl group, a cyano group, a phenyl group, a carboalkoxyl group, a hydroxyl group or an alkoxy group; and  $Z_6$  represents a phenyl group or a substituted phenyl group wherein the substituent is alkyl or alkoxy.

3. A silver halide emulsion according to claim 1 wherein the alkyl group of  $R_1$  to  $R_7$  is methyl, ethyl, n-propyl, iso-propyl, n-butyl or iso-butyl.

4. A silver halide emulsion according to claim 2 wherein the alkyl group of  $R_1$  to  $R_7$  is methyl, ethyl, n-propyl, iso-propyl, n-butyl or iso-butyl.

5. A silver halide emulsion according to claim 1 wherein said substituted alkyl group is a vinylmethyl group, a benzyl group, a  $\beta$ -acetoxethyl group, a  $\gamma$ -acetoxypropyl group, a  $\gamma$ -carboxypropyl group, a  $\beta$ -carboxyethyl group, a  $\gamma$ -sulfatopropyl group, a  $\delta$ -sulfobutyl group, a  $\delta$ -N-acetylsulfamylbutyl group, a  $\beta$ -hydroxyethyl group, a  $\gamma$ -sulfopropyl group, a  $\gamma$ -sulfobutyl group or a  $\delta$ -sulfobutyl group, and wherein said substituted alkyl group having a sulfo group is a 2-(3-sulfopropoxy)ethyl group, a 2[2-(3-sulfopropoxy)ethoxy]ethyl group, or a 2-hydroxy-1-sulfopropyl group.

6. A silver halide emulsion as in claim 2 wherein the total amount of said sensitizing dyes I and II and said compound of formula III is within the range of from  $1 \times 10^{-6}$  mol to  $1 \times 10^{-3}$  mol per mol of silver halide.

7. A silver halide emulsion as in claim 1 wherein said emulsion contains one sensitizing dye of formula I and the following second sensitizing dye:



8. A silver halide emulsion as in claim 2 which contains a second sensitizing dye of the following formula:



at least one first sensitizing dye of formula I and at least one compound of formula III.

9. A photographic light-sensitive element comprising

21

a support having thereon at least one layer containing the photographic silver halide emulsion as in claim 1.

10. A silver halide emulsion according to claim 1 containing one sensitizing dye of formula I and the second sensitizing dye:



11. A silver halide emulsion according to claim 1 containing one sensitizing dye of formula I and the following second sensitizing dye:



12. A silver halide emulsion according to claim 1 containing a sensitizing dye of formula I and a second sensitizing dye of the formula:



13. A silver halide emulsion according to claim 1 containing a sensitizing dye of formula I and a second sensitizing dye of the formula:

3,849,147

22



5

14. A silver halide emulsion according to claim 1 containing one sensitizing dye of formula II and the following sensitizing dye:



15

wherein R<sub>1</sub> and R<sub>2</sub> have the same meaning as in claim 1.

15. A silver halide emulsion according to claim 1 containing one sensitizing dye of formula II and the following sensitizing dye:



20

wherein R<sub>1</sub>, R<sub>2</sub>, R<sub>3</sub> and R<sub>4</sub> have the same meaning as in claim 1.

\* \* \* \* \*

30

50

55

60

65